# EUROPEAN PATENT SPECIFICATION

(11) **EP 2 942 423 B1**
(45) Date of publication and mention of the grant of the patent: **13.02.2019**
(21) Application number: 14861982.8
(22) Date of filing: 11.06.2014
(51) Int. Cl.: C25D 11/04, C25D 11/16, C25D 11/18, C23F 1/20, C23F 3/03, C23C 22/34, C23G 1/12, C25D 11/08, C25D 11/24

(54) **METHOD FOR TREATING SURFACE OF ALUMINUM ALLOY**
VERFAHREN ZUR OBERFLÄCHENBEHANDLUNG EINER ALUMINIUMLEGIERUNG
PROCÉDÉ DE TRAITEMENT DE SURFACE D'ALLIAGE D'ALUMINIUM

(30) Priority: 18.11.2013 KR 20130139920
(43) Date of publication of application: 11.11.2015
(73) Proprietor: Kwang Dong Hitech Co., Ltd, Kwangju-si 506-253 (KR)
(72) Inventor: CHAE, Soo Yoen, Hwaseong-si Gyeonggi-do 445-821 (KR)
(74) Representative: Beck & Rössig European Patent Attorneys
(86) International application number: PCT/KR2014/005119
(87) International publication number: WO 2015/072640

(56) References cited:
- WO-A1-2012/119306
- JP-A- 2001 059 200
- JP-A- 2003 003 295
- KR-A- 20090 051 271
- KR-A- 20090 058 068
- KR-A- 20100 085 704
- US-A- 3 228 816
- US-A1- 2010 183 869

## Description

### Technical Field

The present invention relates to a method of surface-treating an aluminum alloy comprising the features of the preamble portion of claim 1.

### Background Art

Typically, the surface of an aluminum alloy subjected to a rolling or extrusion process includes rough marks, and thus such a rough surface of the aluminum alloy is removed by mechanical grinding and etching.

An anodic oxidation method, which is a metal surface treatment method, is referred to as an alumite process. Specifically, when aluminum or an aluminum alloy is immersed in a solution of sulfuric acid, oxalic acid or chromic acid so as to undergo anodic electrolysis, anodic oxidation occurs, thus forming an anodic oxide film (Al₂O₃ • xH₂O) on the surface of aluminum, ultimately enhancing corrosion resistance and surface hardness of the aluminum alloy.

In addition to the enhancements in corrosion resistance and surface hardness of the aluminum alloy as mentioned above, the anodic oxidation method enables the anodic oxide film to be colored via adsorption with a dye. Hence, this metal surface treatment method is widely useful.

As for conventional anodic oxidation, however, as the anodic oxidation time increases, the surface gloss of the aluminum alloy may decrease. Even when the surface of the aluminum alloy having low gloss is subjected to polishing after anodic oxidation, it is difficult to ensure a high-gloss surface of the aluminum alloy.

With the aim of alleviating these problems, Korean Patent Application Publication No. 10-2005-0118918, entitled "A surface treatment method of aluminum and white-board product thereby", includes a pretreatment process for immersing an aluminum sheet in a mixed aqueous solution of acidic ammonium fluoride and calcium gluconate.

Also, Korean Patent No. 10-0864316, entitled "Method of chemical treatment for surface of aluminum pipe for organic photo conductor drum", discloses an increase in gloss of the aluminum pipe, including immersing the aluminum pipe in a 5 ∼ 20 %(w/v) ammonium fluoride solution containing 0.001 ∼ 0.03 wt% of a hydrofluoric acid additive for 1 ∼ 5 min so as to be acid-etched.

However, when the acidic ammonium fluoride is used alone or in combination in the form of a mixed aqueous solution with calcium gluconate or hydrofluoric acid in this way, a white film may be obtained but may be opaque and dull, making it difficult to ensure a high-gloss surface of the aluminum alloy.

A method of surface-treating an aluminum alloy comprising the features of the preamble portion of claim 1 is known from WO 2012/119306 A1.

Further, US 3,228,816 A1 teaches a three-constituent acid composition for etching and, alternatively, a two-constituent acid composition. The three-constituent acid composition is composed predominately of water with minor portions of nitric, hydrofluoric and boric acids. The two-constituent acid composition is composed predominately of water with minor portions of nitric and fluoboric acids. According to US 3,228,816 A1 the acid composition is critical to both as to the components and their proportions, particularly with respect to the relative concentrations of the fluoride and borate ions, and is also critical as to the range of operating temperatures. Hyperfluoric acid is considered as etchant virgorously attacking aluminum and its alloys while borate acts as passivating agent providing a retarding or inhibiting effect. At temperatures of around 200°F, i.e. 93,3°C, the action on the metal is said to increase but the solution is insufficient to adequately polish the metal. In this context nitric acid is taught as oxidizing agent which comes into play at temperatures above 160°F. For these reasons US 3,228,816 A1 suggests an operating temperature for the disclosed solutions between 160°F and 200°F, i.e 71,1°C to 93,3°C.

### Disclosure

### Technical Problem

Accordingly, the present invention has been made keeping in mind the above problems encountered in the related art, and an object of the present invention is to provide an alternative method of surface-treating an aluminum alloy, wherein scratches and grinding pad marks generated on the surface of an aluminum alloy by mechanical grinding may be effectively removed, and a high-gloss surface of the aluminum alloy may be obtained, regardless of anodic oxidation time.

### Technical Solution

In order to accomplish the above object, the present invention provides a method as defined in claim 1.

Advantageous embodiments are indicated in further claims.

### Advantageous Effects

According to the present invention, scratches and grinding pad marks generated on the surface of an aluminum alloy by mechanical grinding can be effectively removed, and a high-gloss surface of the aluminum alloy can be obtained regardless of the anodic oxidation time.

### Description of Drawings

FIG. 1 illustrates a process of surface-treating an aluminum alloy according to an embodiment of the present invention; and
FIG. 2 schematically illustrates the surface of the aluminum or aluminum alloy before (a) and after (b) the third step of FIG. 1.

### Best Mode

The terms used in the present invention are possibly selected from among currently well-known terms, some of the terms mentioned in the description of the present invention have been selected by the applicant, the detailed meanings of which should be understood not simply by the actual terms used but by the meaning of each term in the detailed description of the invention or in consideration of the meanings used.

Hereinafter, a detailed description will be given of the technical construction of the present invention with reference to preferred embodiments illustrated in the appended drawings.

In regard thereto, FIG. 1 illustrates a process of surface-treating an aluminum alloy according to an embodiment of the present invention, and FIG. 2 schematically illustrates the surface of the aluminum alloy before (a) and after (b) the third step of FIG. 1.

As illustrated in FIGS. 1 and 2, the method of surface-treating an aluminum alloy according to an embodiment of the present invention includes pretreating aluminum or an aluminum alloy prepared by extrusion or rolling.

As such, such pretreatment includes grinding the surface of the prepared aluminum alloy (S100) and immersing the ground aluminum alloy in a degreasing solution having a predetermined composition, thus degreasing the surface of the aluminum alloy to remove impurities therefrom (S200).

Below is a description of these pretreatment steps (S100 and S200) .

Grinding the surface of the aluminum alloy (S100) is a step (S100) of mechanically grinding the prepared aluminum or aluminum alloy using a variety of grinding agents including oil or fat grinding agents by means of any grinder, but the present invention is not particularly limited thereto.

After the step (S100) of grinding the surface of the aluminum alloy, impurities or grinding agent may remain on the surface of the aluminum or aluminum alloy due to the mechanical grinding. These impurities have to be removed.

In order to remove any impurities or remaining grinding agent, the method of surface-treating the aluminum alloy according to the embodiment of the present invention includes immersing the ground aluminum or aluminum alloy in a degreasing solution having a predetermined composition, and thereby the impurities or remaining grinding agent on the surface of the aluminum or aluminum alloy are removed by degreasing (S200).

As such, removing the impurities or remaining grinding agent by degreasing (S200) may be performed in such a manner that the impurities or remaining grinding agent are removed from the surface of the aluminum or aluminum alloy using a degreasing solution including various nonionic surfactants and sulfuric acid (H₂SO₄).

In a preferred embodiment of the present invention, the degreasing solution is prepared by mixing 1 L of water with 3 ∼ 10% of alkylamine ethoxylate or alcohol ethoxylate and 3 ∼ 10% of sulfuric acid based on the total weight thereof.

The aluminum or aluminum alloy is immersed in the degreasing solution under various temperatures and time conditions, thus removing the impurities or remaining grinding agent. In a preferred embodiment of the present invention, the aluminum or aluminum alloy is immersed in the degreasing solution at 50 ∼ 60°C for 3 ∼ 10 min to remove any impurities or remaining grinding agent.

Also, removing the impurities or remaining grinding agent by degreasing (S200) may be effectively implemented by applying ultrasonic waves or vibration to the aluminum or aluminum alloy, which is immersed in the degreasing solution, or by shaking the degreasing solution.

Meanwhile, the aluminum or aluminum alloy prepared by rolling or extrusion has a rough surface due to the nature of the corresponding process. As such, limitations are imposed on the removal of such a rough surface by the mechanical grinding step (S100) and the degreasing step (S200).

Specifically, the rough surface may be removed to some extent by the mechanical grinding step (S100) and the degreasing step (S200). As illustrated in FIG. 2(a), however, fine grinding pad marks or scratches may be present after the degreasing step (S200).

Even when the surface of the aluminum or aluminum alloy including such fine grinding pad marks or scratches is further subjected to anodic oxidation and polishing, it is difficult to obtain a high-gloss surface.

After the degreasing step (S200), in order to remove fine grinding pad marks or scratches from the surface of the aluminum or aluminum alloy, the method of surface-treating the aluminum alloy according to the embodiment of the present invention includes immersing the aluminum or aluminum alloy in an etching solution having a predetermined composition, and thereby the fine grinding pad marks or scratches existing on the surface of the aluminum or aluminum alloy may be removed by etching, and simultaneously, a transparent glossy film as illustrated in FIG. 2(b) is formed (S300).

According to the present invention, the etching solution is prepared by heat-dissolving 45 ∼ 475 g of acidic ammonium fluoride in a mixed solution resulting from mixing 1 L of water and 1 ∼ 9% of boric acid based on the total weight thereof.

The acidic ammonium fluoride may be any one selected from among NH₄F, NH₄HF and NH₄HF₂, and the boric acid is preferably ortho-boric acid that is represented by H₃BO₃ and is colorless, transparent or lustrous.

The reason why the etching solution comprising acidic ammonium fluoride and boric acid as above is used is as follows: when using a conventional etching solution comprising an acidic ammonium fluoride aqueous solution or a mixed aqueous solution of acidic ammonium fluoride and calcium gluconate or hydrofluoric acid, it is possible to obtain the surface of aluminum or an aluminum alloy without fine grinding pad marks or scratches.

However, when the surface of the aluminum or aluminum alloy is etched using such a conventional etching solution, it may become opaque and dull, thereby making it difficult to obtain a high-gloss surface of the aluminum or aluminum alloy. Hence, the etching solution comprising acidic ammonium fluoride and boric acid is useful.

Furthermore, forming the transparent glossy film (S300) may be performed under various temperature and time conditions.

According to the present invention, forming the transparent glossy film (S300) is conducted by immersing the aluminum or aluminum alloy in the etching solution at room temperature (about 25°C) for 1 ~ 10 min.

Also, the method of surface-treating the aluminum alloy according to the embodiment of the present invention includes subjecting the aluminum or aluminum alloy having the transparent glossy film to anodic oxidation, thus forming an oxide film at a predetermined thickness on the surface of the aluminum or aluminum alloy (S400).

Forming the oxide film (S400) may be implemented using an electrolytic solution comprising any one or a mixture of two or more selected from among sulfuric acid, oxalic acid and chromic acid.

In a preferred embodiment of the present invention, sulfuric acid (H₂SO₄) is used for the electrolytic solution to enhance profitability, transparency of the oxide film, corrosion resistance, and wear resistance. The aluminum alloy is immersed in the sulfuric acid electrolytic solution at 20°C and a voltage of 14 V is then applied for 50 min, thus forming a 20 ∼ 22 µm thick oxide film.

After the step (S400) of forming the oxide film, the method of surface-treating the aluminum alloy according to the embodiment of the present invention includes post-treating the aluminum or aluminum alloy.

As such, post-treatment may include coloring and polishing the surface of the aluminum alloy having the oxide film (S500) and sealing the colored and polished aluminum alloy (S600).

The aluminum or aluminum alloy may be variously colored via the coloring and polishing (S500), and the polishing process may be performed using any mechanical means, but the present invention is not limited thereto.

After the step (S500) of coloring and polishing, the method of surface-treating the aluminum alloy according to the embodiment of the present invention may include sealing the aluminum or aluminum alloy (S600).

The sealing step (S600) indicates a process of sealing micropores of the oxide film formed by anodic oxidation to thus modify the properties including corrosion resistance, etc.

The sealing step (S600) according to the embodiment of the present invention may be conducted using various sealing processes such as sealing by hydration, metal salt sealing and organic compound sealing.

In a preferred embodiment of the present invention, the sealing step (S600) is performed via metal salt sealing by immersing the aluminum or aluminum alloy having the oxide film in a metal salt aqueous solution.

As such, nickel is used for the metal salt, and the aluminum or aluminum alloy is immersed in a nickel salt aqueous solution at 60 ∼ 80°C for 10 min, thus ensuring a high-gloss surface of the aluminum or aluminum alloy.

According to the embodiment or the preferred embodiment of the present invention, the method of surface-treating the aluminum alloy enables scratches and grinding pad marks generated on the surface of the aluminum or aluminum alloy by mechanical grinding to be effectively removed via the aforementioned steps.

Regardless of the anodic oxidation time, a high-gloss surface of the aluminum alloy may be obtained.

The preferred embodiment of the present invention has been disclosed for illustrative purposes, while those skilled in the art will appreciate that various modifications, additions and substitutions are possible.

### Mode for Invention

Below is a detailed description of an embodiment of the present invention in conjunction with FIGS. 1 and 2.

Referring to FIGS. 1 and 2, a method of surface-treating an aluminum alloy according to an embodiment of the present invention includes pretreating aluminum or an aluminum alloy prepared by extrusion or rolling.

As such, the pretreating process includes grinding the surface of the prepared aluminum alloy (S100) and immersing the ground aluminum alloy in a degreasing solution having a predetermined composition to remove impurities remaining on the surface of the aluminum alloy by degreasing (S200).

These pretreatment steps (S100 and S200) are described in detail below.

Specifically, grinding the surface of the aluminum alloy (S100) is a step (S100) of mechanically grinding the prepared aluminum or aluminum alloy using a variety of grinding agents including oil or fat grinding agents.

After the step (S100) of grinding the surface of the aluminum alloy, impurities or grinding agent may be left behind on the surface of the aluminum or aluminum alloy due to the mechanical grinding. There is a need to remove these remaining impurities.

With the goal of removing the impurities or remaining grinding agent, immersing the ground aluminum or aluminum alloy in a degreasing solution having a predetermined composition is performed, so that the surface of the aluminum or aluminum alloy is degreased to remove the impurities or remaining grinding agent therefrom (S200).

As such, removal of the impurities or remaining grinding agent by degreasing (S200) may be carried out by removing the impurities or remaining grinding agent from the surface of the aluminum or aluminum alloy using a degreasing solution including a nonionic surfactant and sulfuric acid (H₂SO₄).

In the present invention, the degreasing solution may be prepared by mixing 1 L of water with 6.5% of alkylamine ethoxylate or alcohol ethoxylate and 6.5% of sulfuric acid on the total weight thereof.

The aluminum or aluminum alloy is immersed in the degreasing solution at 55°C for 6 min, thus removing the impurities or remaining grinding agent.

Also, removing the impurities or remaining grinding agent by degreasing (S200) may be effectively implemented by applying ultrasonic waves or vibration to the aluminum or aluminum alloy, which is immersed in the degreasing solution, or by shaking the degreasing solution.

Meanwhile, the aluminum or aluminum alloy prepared by rolling or extrusion has a rough surface due to the nature of the corresponding process. As such, the removal of such a rough surface by the mechanical grinding step (S100) and the degreasing step (S200) is limited.

Specifically, the rough surface may be removed to some extent by the mechanical grinding step (S100) and the degreasing step (S200). As illustrated in FIG. 2(a), however, fine grinding pad marks or scratches may be present after the degreasing step (S200).

Even when the surface of the aluminum or aluminum alloy including such fine grinding pad marks or scratches is further subjected to anodic oxidation and polishing, it is difficult to obtain a high-gloss surface.

After the degreasing step (S200), therefore, immersing the aluminum or aluminum alloy in an etching solution having a predetermined composition to remove fine grinding pad marks or scratches from the surface of the aluminum or aluminum alloy is performed, so that the fine grinding pad marks or scratches existing on the surface of the aluminum or aluminum alloy are removed by etching, and simultaneously, a transparent glossy film as illustrated in FIG. 2(b) is formed (S300).

According to the embodiment of the present invention, the etching solution may be prepared by heat-dissolving 260 g of acidic ammonium fluoride in a mixed solution resulting from mixing 1 L of water and 5% of boric acid based on the total weight thereof.

The acidic ammonium fluoride may include NH₄F, and the boric acid may be ortho-boric acid that is represented by H₃BO₃ and is colorless, transparent or lustrous.

The reason why the etching solution comprising acidic ammonium fluoride and boric acid as above is used is as follows: when using a conventional etching solution comprising an acidic ammonium fluoride aqueous solution or a mixed aqueous solution of acidic ammonium fluoride and calcium gluconate or hydrofluoric acid, it is possible to obtain the surface of aluminum or an aluminum alloy without fine grinding pad marks or scratches.

However, when the surface of the aluminum or aluminum alloy is etched using such a conventional etching solution, it may become opaque and dull, making it difficult to afford a high-gloss surface of the aluminum or aluminum alloy. Hence, the etching solution comprising acidic ammonium fluoride and boric acid is useful.

Furthermore, forming the transparent glossy film (S300) may be performed by immersing the aluminum or aluminum alloy in the etching solution at room temperature (25°C) for 5 min.

Then, subjecting the aluminum or aluminum alloy having the transparent glossy film to anodic oxidation to form an oxide film at a predetermined thickness on the surface of the aluminum or aluminum alloy (S400) is performed.

As such, forming the oxide film (S400) may be carried out using an electrolytic solution comprising sulfuric acid.

The aluminum alloy is immersed in the sulfuric acid electrolytic solution at 20°C, followed by applying a voltage of 14 V for 50 min, thus forming a 20 µm thick oxide film.

After the step (S400) of forming the oxide film, post-treating the aluminum or aluminum alloy is conducted.

As such, post-treatment may include coloring and polishing the surface of the aluminum alloy having the oxide film (S500) and sealing the colored and polished aluminum alloy (S600).

After the step (S500) of coloring and polishing, sealing the aluminum or aluminum alloy (S600) is carried out.

The sealing step (S600) is conducted via metal salt sealing in such a manner that the aluminum or aluminum alloy having the oxide film is immersed in a metal salt aqueous solution.

As such, nickel is used for the metal salt, and the aluminum or aluminum alloy is immersed in a nickel salt aqueous solution at 70°C for 10 min, thereby ensuring a high-gloss surface of the aluminum or aluminum alloy.

Consequently, the aforementioned steps of the method of surface-treating the aluminum alloy according to the present invention are effective at removing scratches and grinding pad marks generated on the surface of the aluminum or aluminum alloy by mechanical grinding.

Moreover, the aluminum alloy may have a high-gloss surface, regardless of the anodic oxidation time.

### Industrial Applicability

According to the present invention, a method of surface-treating an aluminum alloy can effectively remove scratches and grinding pad marks generated by mechanical grinding.

Also, regardless of anodic oxidation time, an aluminum alloy having high gloss can be manufactured, and thus the present invention is industrially applicable.

## Claims

1. A method of surface-treating an aluminum alloy, comprising:
pretreating an aluminum alloy;
immersing the pretreated aluminum alloy in an etching solution having a predetermined composition so that a surface of the aluminum alloy is etched, thus forming a transparent glossy film;
subjecting the aluminum alloy having the transparent glossy film to anodic oxidation, thus forming an oxide film on the surface of the aluminum alloy; and
post-treating the aluminum alloy having the oxide film;
**characterised in that**
the etching solution is prepared by heat-dissolving 45 ∼ 475 g of acidic ammonium fluoride in a mixed solution resulting from mixing 1 L of water and 1 ∼ 9% of boric acid based on a total weight thereof, and the aluminum alloy is etched by being immersed in the etching solution at room temperature for 1 ∼ 10 min.

2. The method of claim 1, wherein pretreating the aluminum alloy comprises:
grinding the surface of the aluminum alloy; and
immersing the ground aluminum alloy in a degreasing solution having a predetermined composition to remove impurities from the surface of the aluminum alloy.

3. The method of claim 2, wherein the degreasing solution is prepared by mixing 1 L of water and 3 ∼ 10% of alkylamine ethoxylate or alcohol ethoxylate and 3 ∼ 10% of sulfuric acid based on a total weight thereof, and the aluminum alloy is degreased by being immersed in the degreasing solution at 50 ∼ 60°C for 3 ∼ 10 min.

4. The method of one of claims 1 to 3, wherein forming the oxide film is performed by immersing the aluminum alloy in a sulfuric acid electrolytic solution at 20°C and then applying a voltage of 14 V for 50 min to form the oxide film having a thickness of 20 ∼ 22 µm.

5. The method of one of claims 1 to 4, wherein post-treating the aluminum alloy having the oxide film comprises:
coloring and polishing the surface of the aluminum alloy having the oxide film; and
sealing the colored and polished aluminum alloy.

## Patentansprüche

1. Verfahren zur Oberflächenbehandlung einer Aluminiumlegierung, umfassend:
Vorbehandeln einer Aluminiumlegierung;
Eintauchen der vorbehandelten Aluminiumlegierung in eine Ätzlösung mit einer vorgegebenen Zusammensetzung, so dass eine Oberfläche der Aluminiumlegierung geätzt wird und dadurch ein transparenter Glanzfilm entsteht;
Unterziehen der Aluminiumlegierung mit dem transparenten Glanzfilm einer anodischen Oxidation, so dass eine Oxidschicht auf der Oberfläche der Aluminiumlegierung entsteht; und
Nachbehandeln der Aluminiumlegierung mit der Oxidschicht;
**dadurch gekennzeichnet, dass**
die Ätzlösung durch Auflösen unter Erwärmung von 45 ∼ 475 g von saurem Ammoniumfluorid in einer gemischten Lösung hergestellt wird, die durch Mischen von 1 l Wasser und 1 ∼ 9 % Borsäure, basierend auf einem Gesamtgewicht davon, erhalten wird, und die Aluminiumlegierung durch Eintauchen in die Ätzlösung bei Raumtemperatur für 1 bis 10 Min geätzt wird.

2. Verfahren nach Anspruch 1, wobei das Vorbehandeln der Aluminiumlegierung umfasst:
Schleifen der Oberfläche der Aluminiumlegierung; und
Eintauchen der geschliffenen Aluminiumlegierung in eine Entfettungslösung mit einer vorgegebenen Zusammensetzung, um Verunreinigungen von der Oberfläche der Aluminiumlegierung zu entfernen.

3. Verfahren nach Anspruch 2, wobei die Entfettungslösung durch Mischen von 1 1 Wasser und 3 ∼ 10 % Alkylaminethoxylat oder Alkoholethoxylat und 3 ∼ 10 % Schwefelsäure basierend auf einem Gesamtgewicht davon hergestellt wird, und die Aluminiumlegierung durch Eintauchen in die Entfettungslösung bei 50 ∼ 60°C für 3 ∼ 10 Min entfettet wird.

4. Verfahren nach einem der Ansprüche 1 bis 3, wobei das Bilden der Oxidschicht durch Eintauchen der Aluminiumlegierung in eine Schwefelsäure-Elektrolytlösung bei 20 °C und anschließendes Anlegen einer Spannung von 14 V für 50 Minuten durchgeführt wird, um die Oxidschicht mit einer Dicke von 20 ∼ 22 µm zu bilden.

5. Verfahren nach einem der Ansprüche 1 bis 4, wobei das Nachbehandeln der Aluminiumlegierung mit der Oxidschicht umfasst:
Färben und Polieren der Oberfläche der Aluminiumlegierung mit der Oxidschicht; und
Versiegeln der gefärbten und polierten Aluminiumlegierung.

## Revendications

1. Procédé de traitement de surface d'un alliage d'aluminium, comprenant les étapes suivantes :
pré-traiter un alliage d'aluminium ;
immerger l'alliage d'aluminium pré-traité dans une solution de gravure ayant une composition prédéterminée de sorte qu'une surface de l'alliage d'aluminium soit gravée, formant ainsi un film brillant transparent ;
soumettre l'alliage d'aluminium présentant le film brillant transparent à une oxydation anodique, formant ainsi un film d'oxyde sur la surface de l'alliage d'aluminium ; et
post-traiter l'alliage d'aluminium présentant le film d'oxyde ;
**caractérisé en ce que**
la solution de gravure est préparée par dissolution thermique de 45 à 475 g environ de fluorure d'ammonium acide dans une solution mélangée résultant du mélange de 1 l d'eau et de 1 à 9 % environ d'acide borique sur la base d'un poids total de celle-ci, et l'alliage d'aluminium est gravé en étant immergé dans la solution de gravure à température ambiante pendant environ 1 à 10 min.

2. Procédé selon la revendication 1, dans lequel le pré-traitement de l'alliage d'aluminium comprend les étapes suivantes :
broyer la surface de l'alliage d'aluminium ; et
immerger l'alliage d'aluminium broyé dans une solution de dégraissage ayant une composition prédéterminée pour retirer les impuretés de la surface de l'alliage d'aluminium.

3. Procédé selon la revendication 2, dans lequel la solution de dégraissage est préparée en mélangeant 1 l d'eau et de 3 à 10% environ d'éthoxylate d'alkylamine ou d'éthoxylate d'alcool et de 3 à 10 % environ d'acide sulfurique sur la base d'un poids total de celle-ci, et l'alliage d'aluminium est dégraissé en étant immergé dans la solution de dégraissage à une température comprise entre 50 et 60°C environ pendant 3 à 10 min environ.

4. Procédé selon l'une des revendications 1 à 3, dans lequel la formation du film d'oxyde est réalisée en immergeant l'alliage d'aluminium dans une solution électrolytique d'acide sulfurique à 20°C puis en appliquant une tension de 14 V pendant 50 min pour former le film d'oxyde ayant une épaisseur comprise entre 20 et 22 µm environ.

5. Procédé selon l'une des revendications 1 à 4, dans lequel le post-traitement de l'alliage d'aluminium présentant le film d'oxyde comprend les étapes suivantes :
colorer et polir la surface de l'alliage d'aluminium présentant le film d'oxyde ; et
sceller l'alliage d'aluminium coloré et poli.
